

# UNITED STATES PATENT OFFICE.

THOMAS W. SMILLIE, OF WASHINGTON, DISTRICT OF COLUMBIA.

## MUSIC SHEET OR PAPER FOR MECHANICALLY-OPERATED MUSICAL INSTRUMENTS.

No 827,128.

Specification of Letters Patent.

Patented July 31, 1906.

Application filed January 27, 1904. Serial No. 190,882.

*To all whom it may concern:*

Be it known that I, THOMAS W. SMILLIE, a citizen of the United States, residing at Washington, in the District of Columbia, have invented new and useful Improvements in Music Sheets or Papers for Mechanically-Operated Musical Instruments, of which the following is a specification.

This invention relates to perforated music sheets or papers treated either before or after they have been provided with note-perforations to render them impervious to atmospheric influences.

It is a well-known fact that perforated music sheets or papers employed in connection with self-playing musical instruments respond more or less freely to atmospheric changes and expand and contract in width under the influences of moisture and heat or extreme dryness, which expansion and contraction is sometimes fatal to a proper rendition of the musical composition represented by the note-perforations in the sheet. In use these music-sheets are wound upon removable wooden spools having fixed end flanges, the distance between the flanges being about equal to the width of the music-sheets, and the sheets are wound from these spools onto another spool or roll known as the "take-up," the latter forming a part of the musical instrument, and in passing from one spool to the other the music-sheet passes over a "tracker" or other "note-selecting device" which co-operates with the perforations to actuate the sound-producing mechanism. It will be obvious, therefore, if the music-sheet expands in width to any considerable extent, the opposite longitudinal edges thereof will be brought to bear too much upon the end flanges of the spool, which will tend to bend, crumple, and tear said edges, and as it is absolutely necessary that the music-sheets shall be accurately and evenly guided over the tracker or other note-selecting device in order to secure a proper register of the note-perforations with the tracker-ducts or equivalent elements this crumpling or tearing of the edges of the sheets will render such guiding and register uncertain and unreliable, and will interfere with the proper rendition of the musical composition. This is due to the fact that the sheets are thus made considerably narrower in width than the spools on which they are wound and rewound, and hence they will not wind evenly.

Heretofore and prior to my invention it has been proposed to overcome the above objections by making the spool-flanges laterally adjustable, and also by making the spools themselves of paper, so that they would expand and contract alike with the music-sheets; but these devices are not entirely satisfactory and have never gone into general use, and, besides, they are not directed to the seat of difficulty or trouble.

It is the purpose of my present invention to overcome the before-mentioned objections by treating the music sheet or paper itself, either before or after the same has been perforated, with a composition that will render the paper impervious to atmospheric influences, so that when the sheet is once correctly perforated and fitted to the spools it will remain so permanently, resisting all atmospheric changes. This composition consists of the following ingredients combined in or about the proportions mentioned: gasoline, naphtha, benzin, or other similar solvents, about one quart; paraffin, wax, or other substance of the same nature, one ounce; raw linseed - oil or other suitable bland non-drying oleaginous agent, three-fourth ounce.

The proportions of the above constituents may, of course, be varied to suit the varying weight or sizing of the paper, but it must be understood that they are not to be varied to such an extent as to destroy the softness and flexibility of the paper, which is a necessary element in perforated music-sheets.

The composition, which is in liquid form, is placed in a suitable pan or tray and the music-sheet passed or drawn therethrough, so that both sides thereof will be treated, and the sheet is then dried either naturally or artificially. The gasoline, benzin, or like solvent is employed as a vehicle to carry the other ingredients into the paper. The paraffin or other wax acts as the moisture-repelling medium and prevents the sheet from being affected by atmospheric changes, and the raw linseed or other bland non-drying oleaginous agent keeps the sheet soft and pliable. It is recognized here that raw linseed oil is not of itself, strictly speaking, a non-drying oil, but when combined with paraffin or like waxy substance and not mixed with any of the oxids of lead it becomes for all the practical purposes of this invention a non-drying oil.

Music-sheets treated in the above manner

will not only be impervious to atmospheric influences, but the composition will prevent the wearing of the sheet by friction and act somewhat as a lubricant, thus allowing the same to glide smoothly and freely over the tracker.

A serious objection now present in perforated music-sheets arises from the fact that the paper ordinarily employed wears away during use, which allows the fibers so loosened to be drawn into the tracker-ducts and also into the tubes leading to the pneumatic action, thereby clogging or choking these parts and rendering the same non-responsive. This objection is entirely overcome by my present method of treating the same. Again, the sheets when cut are sometimes ragged at the edges and around the perforations, and these ragged edges gradually wear away during the passage of the sheet over the tracker, allowing the loosened fibers to be drawn into the tracker-ducts, as above set forth. By treating a perforated sheet with the composition herein set forth these ragged edges will be so strengthened that the fibers will not readily wear away.

The music-sheets may be treated with my improved composition either before or after the perforating operation; but I prefer to treat the completed sheet, for in this manner the ragged edges will be strengthened, as before mentioned.

I have found from experiment that perforated music-paper already used in the library and expanded by moisture when treated ac-

cording to my invention will subside to its original size and roll perfectly.

Having thus described my invention, what I claim, and desire to secure by Letters Patents Patent, is—

1. As a new article of manufacture, a sheet of music-paper for use in automatically-operated players, consisting of a strip of thin flexible paper treated with a non-drying composition embodying paraffin or a like substance and a bland oil, the ingredients named being incorporated in the sheet in such proportions as to render the same soft and pliable and non-responsive to atmospheric changes. 40 45

2. As a new article of manufacture, a perforated music-sheet for use in automatically-operated playing devices, consisting of a strip of thin flexible paper treated with a composition comprising a volatile vehicle having incorporated therein a waxy substance and a non-drying oleaginous agent, the ingredients named being incorporated in the sheet in about the proportions stated so as to render the sheet soft and pliable and non-responsive as to expansion and contraction to atmospheric changes. 50 55 60

In testimony whereof I have hereunto set my hand in presence of two subscribing witnesses.

THOMAS W. SMILLIE.

Witnesses:

J. GRANVILLE MEYERS, Jr.,  
GERTRUDE M. STUCKER.